

1

3,336,227

**POLYALKYLENE GLYCOL - DIORTHOSILICIC ACID ESTER LUBRICANTS AND POWER TRANSMITTING FLUIDS**

Herbert Göthel, Oberhausen-Sterkrade, Hans Feichtinger, Dinslaken, and Heinz Noeske, Oberhausen-Sterkrade-Nord, Germany, assignors to Ruhrchemie Aktiengesellschaft, Oberhausen-Holten, Germany, a corporation of Germany

No Drawing. Filed July 8, 1965, Ser. No. 470,629  
Claims priority, application Germany, July 10, 1964,

R 38,337  
20 Claims. (Cl. 252—49.6)

This invention relates to new and useful synthetic liquid compositions or oils. More particularly, the invention is concerned with fluid or oily compositions comprising a diorthosilicic acid ester or a mixture containing a diorthosilicic acid ester.

The fluid compositions of this invention may be used alone or admixed with other liquid materials—e.g., fluid bodies such as polyoxyalkyleneglycol-diortho-silicic acid-hexaalkyl esters disclosed in U.S. Patent No. 2,776,307 as electrically insulating fluids, hydraulic fluids, damping fluids, lubricants, etc.

Synthetic lubricants, power transmission fluids, etc., must possess a number of properties in order to be capable of heavy duty service under varying operating conditions. Such fluids must be characterized by small changes in viscosity with temperature, remain fluid at low temperatures, be non-volatile at high temperatures, have high thermal and oxidative stability, and the lubricating films formed therefrom must have adequate load carrying capacities.

Silicic acid esters are known which more or less meet the above requirements, as, for instance, polyoxyalkyleneglycol-diorthosilicic acid-hexa-alkyl esters disclosed in U.S. Patent No. 2,776,307. However, the viscosity indices of these esters decrease in those instances where the esters have alkyl groups which contain more than 8 carbon atoms. The esters having low viscosity indices are not satisfactory for application as jet propulsion engine oils.

An object of the present invention is to provide silicic acid esters having high boiling ranges, low volatilities, high viscosity indices, low viscosities at low temperatures and as well capable of forming lubricating films having satisfactory load carrying capacities.

Another object of this invention is to provide fluid compositions suitable for use as electrically insulating fluids, hydraulic fluids, damping fluids, lubricants, etc.

Still another object of this invention is to provide fluid compositions suitable for use as electrically insulating fluids, hydraulic fluids, damping fluids, lubricants, etc., comprising a polyalkyleneglycol-diorthosilicic acid-(polyoxyalkyleneglycol-ether)-ester per se or in admixture with other liquid materials, e.g., fluid bodies constituting hydraulic fluids, lubricants, and the like.

These and other objects will be apparent from a consideration of the instant disclosure and claims appended hereto.

In accordance with the present invention it has now been found that liquid material comprising diorthosilicic acid esters of the formula



wherein A represents a polyoxyalkylene radical having 1

2

to 6 and preferably 2 to 4 ether-oxygen atoms, R represents a polyoxyalkylene glycol ether radical having 2 to 8 ether-oxygen atoms, R' represents an alkyl group having 9 to 20 carbon atoms, n is of the class consisting of from 1 to 4 and 0 and wherein R' and R may be the same or different, provides liquid or fluid compositions which are suitable for use as lubricants, brake fluids, hydraulic fluids, etc.

A preferred group of diorthosilicic acid esters for the purposes of the invention has the following formulae:



wherein A, R and R' are as previously defined.

The diorthosilicic acid esters according to the invention have hitherto not been described. They may be prepared by the conventional methods employed in the production of diorthosilicic acid esters.

The advantages of the novel diorthosilicic acid esters of the invention as lubricants and power transmission fluids are shown in the following table wherein a comparison of certain of the esters of the invention with certain known silicic acid esters having similar molecular sizes has been set out. The known esters employed in comparison include di- and tri-oxyalkyleneglycol-diorthosilicic acid-hexa-isodecyl-ester (I, III) as well as tri-oxyalkyleneglycol-diorthosilicic acid-hexa-iso-tridecyl-ester (VIII) corresponding to the formula:



The esters of the invention used in the comparison are the following:

- (II) diethyleneglycol-di-orthosilicic acid-hexa-(diethyleneglycol-n-butyl-ether)-ester
- (VI) diethyleneglycol-di-orthosilicic acid-tri-(diethyleneglycol-ethyl-ether)-tri-(diethyleneglycol-n-butyl-ether)-ester
- (IV) triethyleneglycol-di-orthosilicic acid-hexa-(diethyleneglycol-n-butyl-ether)-ester
- (V) triethyleneglycol-di-orthosilicic acid-tri-(diethyleneglycol-ethyl-ether)-tri-(diethyleneglycol-n-butyl-ether)-ester
- (VII) triethyleneglycol-di-orthosilicic acid-tri-(diethyleneglycol-n-butyl-ether)-tri-(iso-decyl)-ester
- (IX) triethyleneglycol-di-orthosilicic acid-tri-(diethyleneglycol-n-butyl-ether)-tri-(iso-tridecyl)-ester

The expressions Oxo— $C_{10}H_{21}$  and Oxo— $C_{13}H_{27}$  as used in the table designate radicals of alcohols obtained from trimer- or tetramer-propylene by hydroformylation (oxo synthesis) followed by hydrogenation of the hydroformylation product.

The load carrying capacity of the lubricating film of each of the esters was determined using the four-ball testing apparatus as described by Boerlage (Lexikon der Schmiertechnik, G. Voegtle, Franckh'sche Verlagshandlung Stuttgart 1964).

In the table, two numbers are set out under the column "Welding Value." The first number represents the highest possible load in kg. which the lubricating film withstands

for one minute, without alteration, while the second number designates the load at which the balls are welded, i.e., frozen together.

inertness to broad temperatures changes is desirable or required.

When the viscosity of an oil changes only slightly as

TABLE I

| No.  | Di-orthosilicic acid esters                                                      |                                                                                                                                                                                                          |                                     | n     | Molec-<br>ular<br>wt. | Viscosity (cst.) in ° C. |        |        |        | Vis-<br>cosity<br>index | Pour<br>point<br>° C. | Welding<br>value<br>load, kg. |
|------|----------------------------------------------------------------------------------|----------------------------------------------------------------------------------------------------------------------------------------------------------------------------------------------------------|-------------------------------------|-------|-----------------------|--------------------------|--------|--------|--------|-------------------------|-----------------------|-------------------------------|
|      | A                                                                                | R                                                                                                                                                                                                        | R'                                  |       |                       | 98.9                     | 37.8   | -40    | -54    |                         |                       |                               |
| I    | CH <sub>2</sub> CH <sub>2</sub> OCH <sub>2</sub> CH <sub>2</sub>                 |                                                                                                                                                                                                          | Oxo-C <sub>10</sub> H <sub>21</sub> | 6     | 1,102                 | 5.19                     | 22.6   | 3,680  | 26,200 | 167                     | -69                   | 160/170                       |
| II   | CH <sub>2</sub> CH <sub>2</sub> OCH <sub>2</sub> CH <sub>2</sub>                 | (CH <sub>2</sub> CH <sub>2</sub> O) <sub>2</sub> -n-C <sub>4</sub> H <sub>9</sub>                                                                                                                        |                                     | 0     | 1,126                 | 3.9                      | 13.5   | 1,273  | 7,490  | 203                     | -71                   | 170/180                       |
| VI   | CH <sub>2</sub> CH <sub>2</sub> OCH <sub>2</sub> CH <sub>2</sub>                 | {(3(CH <sub>2</sub> CH <sub>2</sub> O) <sub>2</sub> CH <sub>2</sub> CH <sub>3</sub> ) <sub>n</sub> -(3(CH <sub>2</sub> CH <sub>2</sub> O) <sub>2</sub> -n-C <sub>4</sub> H <sub>9</sub> ) <sub>m</sub> } |                                     | 0     | 1,042                 | 4.65                     | 16.2   | 1,950  | 17,050 | 206                     | -70                   | 180/190                       |
| III  | (CH <sub>2</sub> CH <sub>2</sub> O) <sub>2</sub> CH <sub>2</sub> CH <sub>2</sub> | Oxo-C <sub>10</sub> H <sub>21</sub>                                                                                                                                                                      | 6                                   | 1,146 | 7.8                   | 34.6                     | 6,580  | 49,000 | 163    | -68                     | 160/170               |                               |
| IV   | (CH <sub>2</sub> CH <sub>2</sub> O) <sub>2</sub> CH <sub>2</sub> CH <sub>2</sub> | (CH <sub>2</sub> CH <sub>2</sub> O) <sub>2</sub> -n-C <sub>4</sub> H <sub>9</sub>                                                                                                                        |                                     | 0     | 1,170                 | 7.0                      | 26.1   | 2,915  | 18,650 | 180                     | -70                   | 180/190                       |
| V    | (CH <sub>2</sub> CH <sub>2</sub> O) <sub>2</sub> CH <sub>2</sub> CH <sub>2</sub> | {(3(CH <sub>2</sub> CH <sub>2</sub> O) <sub>2</sub> CH <sub>2</sub> CH <sub>3</sub> ) <sub>n</sub> -(3(CH <sub>2</sub> CH <sub>2</sub> O) <sub>2</sub> -n-C <sub>4</sub> H <sub>9</sub> ) <sub>m</sub> } |                                     | 0     | 1,086                 | 6.81                     | 24.25  | 3,005  | 24,650 | 185                     | -69                   | 180/190                       |
| VII  | (CH <sub>2</sub> CH <sub>2</sub> O) <sub>2</sub> CH <sub>2</sub> CH <sub>2</sub> | Oxo-C <sub>10</sub> H <sub>21</sub>                                                                                                                                                                      | 3                                   | 1,158 | 6.9                   | 27.5                     | 3,540  | 29,850 | 175    | -65                     | 170/180               |                               |
| VIII | (CH <sub>2</sub> CH <sub>2</sub> O) <sub>2</sub> CH <sub>2</sub> CH <sub>2</sub> | Oxo-C <sub>13</sub> H <sub>27</sub>                                                                                                                                                                      | 6                                   | 1,398 | 9.2                   | 56.0                     | 30,400 | -----  | 138    | -52                     | 160/170               |                               |
| IX   | (CH <sub>2</sub> CH <sub>2</sub> O) <sub>2</sub> CH <sub>2</sub> CH <sub>2</sub> | Oxo-C <sub>13</sub> H <sub>27</sub>                                                                                                                                                                      | 3                                   | 1,284 | 8.98                  | 41.8                     | 11,400 | -----  | 160    | -60                     | 170/180               |                               |

As can be seen from the table, the viscosities of silicic acid esters having approximately equal molecular weights I and II, III and IV, I and V, I and VI, III and VII, and VIII and IX differ greatly. The viscosity indices of the esters II and IV (according to the invention) lie above 200, which is significantly higher than the viscosity index of the hexa-isodecyl-ester I. The viscosity indices of the triethyleneglycol-diorthosilicic acid esters IV and V differ considerably from those of esters I and III, respectively, of comparable molecular size and, namely, by 17 or 18 units, respectively.

While the viscosity indices of hexa-alkyl esters decrease with increasing size of carbon chains of the radicals R (III, VIII) high viscosity indices, i.e., above 180, for the silicic acid esters according to the invention are retained. If three of the six alkyl radicals in the said silicic acid ester molecular are substituted by diethyleneglycol-n-buty-ether radicals (VII, IX), the viscosity index is considerably improved.

The silicic acid esters according to the invention possess satisfactory low temperature viscosities at, for example, -40° and at -54° C. Because of this favorable viscosity-temperature relationship, the esters of the invention are particularly well suited for use as lubricants, additives to lubricants, as well as power transmission fluids, where extremely low temperatures must be encountered.

Although the esters IV and V, containing oxyalkylene-glycol ether residues, are more viscous at 37.8 and 98.9° C. than the known hexa-isodecyl-ester I, they are much more fluid in the cold than the commercially available lubricating oils of different chemical composition used at present for gas turbine airplanes. The known bis-(2-ethyl-hexyl)-sebacic acid ester, for instance, which has at 37.8° C. the same viscosity as ester II, has a cold viscosity of 10,150 cst.

Ester VII, although highly viscous at 37.8 and 98.9° C., has substantially the same viscosity as ester I at extremely low temperatures. Thus, the di-orthosilicic acid esters containing oxyalkylene-glycol-ether radicals in their molecule according to the invention exhibit an unexpectedly great improvement in their viscosity-temperature relationship, their low temperature behavior, as well as an increased load carrying capacity of their lubricating films as compared with the di-orthosilicic acid esters known in the art.

Because of the high load carrying capacity of lubricating film, the esters according to the invention have proved especially useful under the application of high loads of the resulting mixed friction.

Polyoxyalkylene-glycol-diorthosilicic acid-hexaoxyalkylene-ether esters according to the invention have molecular weights below 900 and are especially suitable for use as hydraulic fluids due to their high viscosity indices, their low viscosities at low temperatures and adequate viscosities at high temperatures, i.e., under conditions wherein

a function of the temperature, it likewise exhibits but an extremely small pressure responsivity. This property is of considerable importance for hydraulic fluids. For instance, diethyleneglycol - diorthosilicic acid-hexa-(ethyl-25 eneglycol-n-butyl-ether)-ester (molecular weight 862) has a viscosity index of 218. Its viscosity at -40° and -54° C. amounts to 780 and 3460 cst., respectively, which constitute very low values. Its viscosity at 98.8° C. amounts to 4.1 cst., which is considerably higher than that of the 30 dibasic carboxylic acid esters known in the art.

The esters of this invention can be used alone or in admixture with other liquid materials known in the art as lubricants or power transmission fluids, e.g., mineral lubricants, dicarboxylic acid esters, phosphoric acid esters, 35 organo-silicium compounds of different structure, as well as with conventional oxidation inhibitors and other like conventional additives. For instance, they may be admixed with (1) a liquid dicarboxylic acid ester or with (2) a liquid organo-silicium compound, as, for example, 40 a methyl polysiloxane, or (3) with both a phosphoric acid ester and an oxidation inhibitor. The ester of the invention is present in any admixture in an amount equal to at least 5%, preferably at least 50%, of the resulting admixture.

45 An especially well suited oxidation inhibitor is phenothiazine. It can be added in amounts from 0.1 up to 1.5% by weight, dependant upon the quantity of the lubricant.

Conventional additives for improving the oiliness of the lubricants consisting of or containing the esters of 50 the invention, as for instance tricresylphosphate may be added in amounts from 0.1 up to 3% by weight dependant upon the quantity of the lubricant. It is not however necessary to employ these additives, since the esters according to the invention per se exhibit outstanding lubricating action.

The diorthosilicic acid esters can be prepared, for instance, by reacting stoichiometric mixtures of suitable alcohols and ether alcohols with gaseous SiCl<sub>4</sub> according to the disclosure of German Patent No. 1,142,855 or as 60 disclosed in German patent application R 32,696 IVb/120, Deutsche Auslegeschrift 1,180,359.

The following examples are intended to illustrate the invention and are not to be interpreted as limiting the same.

65

#### Example I

A reaction vessel (a so-called bubble-column reactor) consisting of a vertical glass tube with an internal diameter of 69 mm. and a height of 550 mm. provided with 70 a glass frit (Jena apparatus glass, grain coarseness 2) in its bottom was charged with 121 g. diethyleneglycol and 1122 g. diethyleneglycol-n-butylether, which had previously been dried to a water content below 0.1%. Silicium tetrachloride was applied dropwise from a dosing vessel 75 into an evaporator coil heated at 80° C., which was gas-

tight connected with the said reaction vessel, by a conduit joining the said reaction vessel below the said glass frit. The silicon tetrachloride vapors evolved in the evaporator coil were sucked through the frit under a vacuum of 180 torr. The ascending  $\text{SiCl}_4$  vapors together with the

of the invention to the conventional ester lubricant are shown in the following Table 2, wherein the properties of the two single esters are shown in comparison with those of the ester mixture, hereinafter designated "admixture 50/50 percent by vol."

TABLE 2

|                                                                                               | $d_{40}^{20}$ | Viscosity in cst. at $^{\circ}\text{C}$ . |       |        | Viscosity index | Flame point, $^{\circ}\text{C}$ . | Welding value load in kg. |
|-----------------------------------------------------------------------------------------------|---------------|-------------------------------------------|-------|--------|-----------------|-----------------------------------|---------------------------|
|                                                                                               |               | 98.9                                      | 37.8  | -54    |                 |                                   |                           |
| Bis-3,5,5-trimethylhexyl adipate                                                              | 0.916         | 3.15                                      | 11.86 | 15,720 | 147             | 222                               | 150/160                   |
| Diethyleneglycol-diorthosilicic acid-tri-(diethyleneglycol-n-butylether)-tri-(isodecyl)-ester | 0.969         | 3.9                                       | 14.43 | 10,100 | 188             | 264                               | 170/180                   |
| Admixture, 50/50 percent by vol.                                                              | 0.944         | 3.52                                      | 13.01 | 12,700 | 169             | 238                               | 170/180                   |

hydrogen chloride evolved during the reaction formed a bubble-column of 420 mm. height with the liquid in the reactor. The liquid mixture of said alcohol and ether, which had been preheated to  $40^{\circ}\text{C}$ . was heated up to  $52^{\circ}\text{C}$ . by the heat of reaction. In order to compensate for the decreasing evolution of heat during the reaction the reaction mixture was heated at about  $50^{\circ}\text{C}$ . during the course of the reaction. 357 g.  $\text{SiCl}_4$  were introduced and

20 25 *Example 3*  
70 parts by volume bis-3,5,5-(trimethylhexyl)-adipate were admixed with 30 parts by volume diethyleneglycol-diorthosilicic acid - hexa-(diethyleneglycol-n-butylether)-ester (ester II as hereinbefore mentioned). The properties of the two single esters are shown in comparison with those of the ester mixture, designated "admixture 70/30% by vol." in Table 3.

TABLE 3

|                                    | $d_{40}^{20}$ | Viscosity in cst. at $^{\circ}\text{C}$ . |       |        | Viscosity index | Flame point, $^{\circ}\text{C}$ . | Welding value load in kg. |
|------------------------------------|---------------|-------------------------------------------|-------|--------|-----------------|-----------------------------------|---------------------------|
|                                    |               | 98.9                                      | 37.8  | -54    |                 |                                   |                           |
| Bis-3,5,5-(trimethylhexyl)-adipate | 0.916         | 3.15                                      | 11.86 | 15,720 | 147             | 222                               | 150/160                   |
| Ester II                           | 1.035         | 3.9                                       | 13.5  | 7,490  | 204             | 251                               | 170/180                   |
| Admixture, 70/30 percent by vol.   | 0.952         | 3.4                                       | 12.69 | 11,150 | 163             | 230                               | 170/180                   |

converted during 100 minutes. After termination of the reaction, the reaction vessel was heated at  $110^{\circ}\text{C}$ . for 2 hours whereby dissolved hydrogen chloride was removed from the reaction mixture under introduction of nitrogen at a vacuum of 20 torr. (After the said treatment the Beilstein-reaction was negative.) Thereafter the non-reacted excess amounts of the reactants (125 g.) were distilled off from the reaction product under a vacuum of 0.01 torr up to a temperature of  $196^{\circ}\text{C}$ . As distillation residue 1150 g. of diethyleneglycol-diorthosilicic acid hexa - (diethyleneglycol - n - butylether)ester (density  $d_{40}^{20}=1.038$ , index of refraction  $n_{20}^{D}=1.4452$ ) were obtained. The silicon content of the product ester was determined to 5.02% (calculated 4.98%); the viscosity of the ester at  $98.9^{\circ}\text{C}$ . was 3.9 cst., at  $37.8^{\circ}\text{C}$ . 13.5 cst., at  $-40^{\circ}\text{C}$ . 1273 cst., at  $-54^{\circ}\text{C}$ . 7490 cst.; its viscosity index amounted to 203, its flow point (or setting point) was 71° C.

40 In analogous manner other esters according to the invention can be prepared.

#### Example 2

55 60 50 parts by volume of a dibasic ester known in the art namely bis-3,5,5-trimethylhexyl-adipate were admixed with 50 parts by volume diethyleneglycol-diorthosilicic acid - tri - (diethyleneglycol-n-butylether)-tri-(iso-decyl) ester. The advantages of the admixture of the novel ester

Due to the admixture of the ester of the invention the following properties of dibasic esters, serving as lubricants for turbo-jets are generally improved:

The viscosity in the temperature range above  $50^{\circ}\text{C}$ . is increased, in the temperature range below  $37.8^{\circ}\text{C}$ . decreased. The viscosity index is increased, the flame point and the load carrying capacity are also increased.

#### Example 4

75 parts by volume of a mineral lubricating oil (free of any additive) were admixed with 25 parts by volume diethyleneglycol-diorthosilicic acid-hexa-(diethyleneglycol-n-butylether)-ester (ester II of the invention). A comparison of the lubricant so obtained (hereinafter called admixture 75/25 percent by vol. M) with the said mineral oil and ester II has been set out in Table 4.

#### Example 5

55 60 50 parts by volume of the mineral lubricating oil mentioned in Example 4 were admixed with 50 parts by volume diethyleneglycol-diorthosilicic acid-tri-(diethyleneglycol-n-butylether)-tri-(isodecyl)-ester according to the invention. A comparison of the lubricant so obtained (hereinafter called admixture 50/50 percent by vol. M) with the said mineral oil and the ester according to the invention has also been set out in Table 4.

TABLE 4

|                                                                                               | $d_{40}^{20}$ | Viscosity in cst. at $^{\circ}\text{C}$ . |       |        | Viscosity index | Flame point, $^{\circ}\text{C}$ . | Setting point, $^{\circ}\text{C}$ . |
|-----------------------------------------------------------------------------------------------|---------------|-------------------------------------------|-------|--------|-----------------|-----------------------------------|-------------------------------------|
|                                                                                               |               | 98.9                                      | 37.8  | -17.8  |                 |                                   |                                     |
| Mineral lubricating oil                                                                       | 0.990         | 11.5                                      | 130   | 25,100 | 79              | 238                               | -19                                 |
| Ester II                                                                                      | 1.035         | 3.9                                       | 13.5  | 132    | 204             | 251                               | -72                                 |
| Admixture, 75/25 percent by vol. M                                                            | 1.002         | 9.01                                      | 67.5  | 4,030  | 115             | 241                               | -21                                 |
| Diethyleneglycol-diorthosilicic acid-tri-(diethyleneglycol-n-butylether)-tri-(isodecyl)-ester | 0.969         | 3.9                                       | 14.43 | 152    | 188             | 252                               | -71                                 |
| Admixture, 50/50 percent by vol. M                                                            | 0.979         | 6.4                                       | 34.7  | 2,120  | 136             | 244                               | -23                                 |

The admixture according to Examples 4 and 5 represent motor oils, which meet the demands for several classes according to the SAE-classification (Society of Automotive Engineers).

Due to the addition of the esters of the invention to mineral lubricating oils, essential properties of these oils are improved. The viscosity index is increased (as for instance for 36 units at an addition of 25% of the ester of the invention). The viscosity, especially at low temperatures is diminished. The flame points are raised and the setting points are lowered. Further on, the lubricating action is improved.

We claim:

1. A lubricant and power transmission fluid comprising at least 5% by weight of a diorthosilicic acid ester of the formula:



wherein A represents a polyoxyalkylene radical having 1 to 6 ether oxygen atoms, R represents a polyoxyalkylene-glycol-ether radical having 2 to 8 ether-oxygen atoms, R' represents alkyl having 9 to 20 carbon atoms, and n is of the class consisting of integers of from 1 to 4 and 0 admixed with another liquid lubricant.

2. A lubricant and power transmission fluid according to claim 1 additionally containing an anti-oxidant.

3. A lubricant and power transmission fluid according to claim 1 wherein said diorthosilicic acid ester is



wherein R is as defined in claim 1, and A is a polyoxyalkylene radical having 1 to 6 ether oxygen atoms.

4. A lubricant and power transmission fluid according to claim 1, wherein said diorthosilicic acid ester has the formula:



wherein A, R, and R' are as defined in claim 1.

5. A lubricant and power transmission fluid according to claim 1, wherein said diorthosilicic acid ester is diethyleneglycol - diorthosilicic acid - hexa-(diethyleneglycol-n-butyl-ether)-ester.

6. A lubricant and power transmission fluid according to claim 1, wherein said diorthosilicic acid ester is diethyleneglycol - diorthosilicic acid - tri-(diethyleneglycol-ethyl-ether)-tri-(diethyleneglycol-n-butyl-ether)-ester.

7. A lubricant and power transmission fluid according to claim 1, wherein said diorthosilicic acid ester is triethyleneglycol-diorthosilicic acid-hexa-(diethyleneglycol-n-butyl-ether)-ester.

8. A lubricant and power transmission fluid according to claim 1, wherein said diorthosilicic acid ester is triethyleneglycol - diorthosilicic acid - tri-(diethyleneglycol-ethyl-ether)-tri-(diethyleneglycol-n-butyl-ether)-ester.

9. A lubricant and power transmission fluid according to claim 1, wherein said diorthosilicic acid ester is triethyleneglycol - diorthosilicic acid-tri-(diethyleneglycol-n-butyl-ether)-tri-(iso-decyl)-ester.

10. A lubricant and power transmission fluid according to claim 1, wherein said diorthosilicic acid ester is triethyleneglycol-diorthosilicic acid-tri-(diethyleneglycol-n-butyl-ether)-tri-(iso-tridecyl)-ester.

11. A lubricant and power transmission fluid comprising at least 50% by weight of a diorthosilicic acid ester of the formula:



5 wherein A represents a polyoxyalkylene radical having 1 to 6 ether oxygen atoms, R represents a polyoxyalkylene-glycol-ether radical having 2 to 8 ether-oxygen atoms, R' represents alkyl having 9 to 20 carbon atoms, and n is of the class consisting of integers of from 1 to 4 and 0 admixed with another liquid lubricant.

10 12. A lubricant and power transmission fluid according to claim 11 additionally containing an antioxidant.

13. A lubricant and power transmission fluid according to claim 11 wherein said diorthosilicic acid ester is



wherein A and R are as defined in claim 11.

14. A lubricant and power transmission fluid according to claim 11, wherein said diorthosilicic acid ester has the formula:



wherein A, R and R' are as defined in claim 11.

15. A lubricant and power transmission fluid according to claim 11, wherein said diorthosilicic acid ester is diethyleneglycol - diorthosilicic acid - hexa-(diethyleneglycol-n-butyl-ether)-ester.

20 16. A lubricant and power transmission fluid according to claim 11, wherein said diorthosilicic acid ester is diethyleneglycol - diorthosilicic acid - tri - (diethyleneglycol - ethyl-ether)-tri-(diethyleneglycol-n-butyl-ether)-ester.

25 17. A lubricant and power transmission fluid according to claim 11, wherein said diorthosilicic acid ester is triethyleneglycol - diorthosilicic acid - hexa - (diethyleneglycol-n-butyl-ether)-ester.

30 18. A lubricant and power transmission fluid according to claim 11, wherein said diorthosilicic acid ester is triethyleneglycol - diorthosilicic acid - tri - (diethyleneglycol - ethyl-ether)-tri-(diethyleneglycol-n-butyl-ether)-ester.

35 19. A lubricant and power transmission fluid according to claim 11, wherein said diorthosilicic acid ester is triethyleneglycol - diorthosilicic acid - tri - (diethyleneglycol-n-butyl-ether)-tri-(iso-decyl)-ester.

40 20. A lubricant and power transmission fluid according to claim 11, wherein said diorthosilicic acid ester is triethyleneglycol - diorthosilicic acid - tri - (diethyleneglycol-n-butyl-ether)-tri-(iso-tridecyl)-ester.

#### References Cited

#### UNITED STATES PATENTS

|    |           |         |           |            |
|----|-----------|---------|-----------|------------|
| 60 | 2,724,698 | 11/1955 | Kittleson | 252—49.6   |
|    | 2,947,772 | 8/1960  | Eynon     | 252—49.6 X |
|    | 3,029,269 | 4/1962  | Abbott    | 252—49.6 X |
|    | 3,118,841 | 1/1964  | Moreton   | 252—49.6 X |
|    | 3,133,111 | 5/1964  | Wheeler   | 252—49.6 X |

65 65 DANIEL E. WYMAN, Primary Examiner.

W. H. CANNON, Assistant Examiner.

UNITED STATES PATENT OFFICE  
CERTIFICATE OF CORRECTION

Patent No. 3,336,227

August 15, 1967

Herbert Göthel et al.

It is hereby certified that error appears in the above numbered patent requiring correction and that the said Letters Patent should read as corrected below.

Columns 5 and 6, TABLE 2, third column, line 3 thereof, for "3.52" read -- 3.53 --; column 8, line 27, for "((SOi)<sub>2</sub>(OR)<sub>3</sub>(OR')<sub>3</sub>)<sub>3</sub>" read -- A(OSi)<sub>2</sub>(OR)<sub>3</sub>(OR')<sub>3</sub> --.

Signed and sealed this 15th day of October 1968.

(SEAL)

Attest:

Edward M. Fletcher, Jr.

Attesting Officer

EDWARD J. BRENNER

Commissioner of Patents

UNITED STATES PATENT OFFICE  
CERTIFICATE OF CORRECTION

Patent No. 3,336,227

August 15, 1967

Herbert Göthel et al.

It is certified that error appears in the above identified patent and that said Letters Patent are hereby corrected as shown below:

Columns 3 and 4, TABLE I, under the heading "-54" line 2 thereof "7,490" should read -- 7,940 --.

Signed and sealed this 9th day of December 1969.

(SEAL)

Attest:

Edward M. Fletcher, Jr.

Attesting Officer

WILLIAM E. SCHUYLER, JR.

Commissioner of Patents